# EUROPEAN PATENT SPECIFICATION

(11) **EP 0 065 043 B1**
(45) Date of publication and mention of the grant of the patent: **28.11.1984**
(21) Application number: 81302205.0
(22) Date of filing: 19.05.1981
(51) Int. Cl.: B44C 3/04, B44C 5/04

(54) **Method of imparting color highlights or shadows to a textured decorative laminate.**
Methode zum Verleihen von Licht- oder Schattenfarbeffekten an dekorative, texturierte Schichtstoffe
Méthode pour conférer des effets de couleur en clair ou en ombre à des strafifiés texturés décoratifs

(43) Date of publication of application: 24.11.1982
(73) Proprietor: CONSOLIDATED PAPERS, INC., Wisconsin Rapids Wisconsin 54494 (US)
(72) Inventor: Endrizzi, Gilbert Daniel, Wisconsin Rapids Wisconsin 54494 (US)
(74) Representative: Taylor, Phillip Kenneth

## Description

This invention relates to a method of imparting color highlights or shadows to a textured surface of decorative laminates in the course of production of decorative plastics laminates, which are extensively used in making furniture, counter tops, panelling and other decorative or functional surfaces.

The art of making such laminates is well known. A plurality of sheets of resin impregnated kraft paper are stacked together to form a core or backing. The resin employed is a heat curable type such as phenol formaldehyde. A decorative sheet of paper having a printed design or solid color and impregnated with a melamine resin is laid over the core, and an overlay sheet, usually melamine impregnated alpha cellulose paper, is superimposed over the decorative sheet. In some instances, especially where the final product is of solid color, the overlay sheet may be omitted. A panel of particle board may be substituted for the core sheets.

The foregoing assembly of resin impregnated sheets is subjected to heat and compression by confining the same between heated press plates or molding cauls such that the sheets become firmly adhered to one another as the resin cures. A release sheet composed of relatively non-adhereable paper, plastics film or aluminum foil is interposed between the decorative surface and the caul to prevent adhesion between the caul and the decorative surface.

Various techniques have been developed for applying a textured surface to the decorative surface of such laminates. U.S. Patent No. 1,742,516 describes a process wherein a design or letter is embossed in a laminate by using an engraved caul having the design depossed therein. U.S. Patent No. 1,997,358 and No. 2,133,081 describe the texturizing of plastics laminates utilizing an embossed metal caul.

Inasmuch as engraved or embossed metal cauls are expensive to produce and have a short life span, subsequent efforts have been directed primarily toward substitute methods. U.S. Patent No. 2,606,855 discloses a process of using a master to make a number of textured caul plates from a stack of resin impregnated paper. Similar techniques utilizing embossed or debossed plastics laminates as molding cauls are described in U.S. Patent No. 3,303,081 and No. 3,311,520. U.S. Patent No. 3,373,068 describes the use of particulate matter on the decorative sheet to impart texture thereto.

In U.S. Patent No. 3,616,011 there is described another method for making a textured molding caul wherein a textured original is sandwiched between a pair of thin flexible resin impregnated sheets. The sheets are forced intimately into the surface recesses of the original and the resin is cured. Thereafter, the resin-set sandwich of the original and the sheets are used as a master molding caul.

Often it is desirable to produce a laminate that simulates another product, a good example being a wood grained surface. In such a case, it has been possible to use a decorative sheet having a colored wood grain printed thereon, and the decorative surface may also be textured during the subsequent molding process. It is not usually possible or convenient, however, to impart a texture conforming to the print pattern, and the resulting product does not have the combined texture and appearance of a naturally stained wood wherein the grain is highlighted by differential absorption of the stain into the grain, saw marks or depressed areas of the wood.

The present invention represents a further improvement in the production of textured decorative laminates, which allows for greater realism, warmth and a contrasting textural quality heretofore not attainable.

In the production of a textured decorative laminate, a release sheet having a coating of pigment thereon is applied over the decorative surface before the laminate is pressurized against a textured molding caul. The release sheet may be composed, for example, of a sheet of polymeric material having a thin layer of ink applied substantially uniformly on the surface against which the panel or laminate is to be molded.

As the laminate is pressurized and heated, the pigment is uniformly transferred to the texturized surface, the color of the pigment being selected so as to contrast with the color of the decorative sheet.

After the lamination has been completed, the release sheet is removed to expose a textured surface that is substantially uniformly colored by the pigment. The decorative surface is then subjected to surface rubbing, brushing or light abrasion to the extent necessary to remove color from the raised or embossed portions while allowing more color to remain in the depressed or debossed areas, thus highlighting or shadowing the texture and providing added visual dimension to the appearance of the textured surface.

It is believed that a portion of the transferred pigment is absorbed into the decorative surface during the application of heat and pressure, particularly into the debossed areas, and any pigment not removed by the subsequent rubbing has a high degree of adherence to the product. Equivalent results are not achieved by the application of liquid pigment to the relatively non-porous surface of a finished laminate followed by surface rubbing.

In order to carry out the process of the present invention, any of the well known methods of making textured laminates may be employed. A variety of textures are possible, such as wood grain, fabric, decorative objects, writing or printing, as well as many others. The process of making the textured laminate from a textured caul is conventional, and the present invention resides in imparting color highlights to the textured surface.

The core sheets or other suitable backing, decorative sheet and overlay sheet, as well as the resins used to impregnate such sheets and the processing conditions, follow conventional practices such as described in the foregoing patents. In the conventional process, the core is made up from a plurality of resin impregnated kraft sheets. These sheets are normally impregnated with a phenolic resin, allowed to at least partially dry, and then stacked in a superimposed relation. The number of sheets utilized may vary and ordinarily the number will vary between three and six. Other core materials, such as particle board, may be used. Immediately above the core sheet assembly or backing there is positioned a resin impregnated decorative sheet, which in the case of the preferred embodiment will be a sheet having color, printing, or other decoration thereon, for example, printing that resembles a grained wood panel. Superimposed above the print sheet in many cases is a protective overlay sheet of fine paper such as alpha cellulose. The overlay and print sheet are impregnated with a heat curable resin, preferably with a noble thermosetting resin such as melamine formaldehyde resin or the like. Alternatively, the decorative sheet may be replaced by metal foil.

In accordance with conventional practices, the sandwich of the aforesaid materials is placed between a pair of rigid caul plates. The caul plate facing the decorative sheet is provided with a desired textured surface by any of the well known and conventional methods, and a release sheet is placed between the caul and the outer sheet of the laminate. The assembly is placed in a heated press, and the sandwich is subjected to heat and pressure for a time sufficient to cure the resin in the laminate, i.e. typically 500 to 2,000 p.s.i. (3,447x10³ to 13,790x10³ Pa), 200° to 400°F (93.3° to 204.4°C), and 15 to 60 minutes. The resulting product is a rigid laminate having a hard, durable decorative and textured surface.

In the preferred embodiment, the textured caul is prepared by any suitable method. For example, the caul plate may be a rigid metal plate with any desired texture etched thereon by conventional methods.

Another suitable method for preparing a textured caul plate is described in U.S. Patent No. 3,616,011. As described in this patent, a consumable original textured panel or sheet is sandwiched between a pair of resin impregnated or resin containing overlay sheets of a size slightly larger than the original. The overlay sheets and the curable resin therein may be of any of a wide variety of acceptable materials, such as various heat curable resins, such as melamine, phenolic, epoxy, urea formaldehyde and others. Each of the overlay sheets is covered by a release sheet, and the release sheets in turn may be backed by a stack of padding sheets, such as sheets of kraft paper.

The resulting assembly is then placed in a molding press between a pair of cauls, and the assembly is heated and compressed between the cauls in a conventional manner until the resin is cured. Upon curing, the overlay sheets bond to the textured core and assume the texture of the core. The resulting laminate, which may be textured on one or both sides, is used as a molding caul to make textured decorative laminates, as hereinbefore described.

It should be understood that the method of imparting color highlights in accordance with the present invention is carried out as part of the formation of the textured decorative laminate. Color is applied to the decorative surface during the pressure molding procedure, and any excess color is removed from the textured surface after completion of the molding operation.

In carrying out the process of the present invention, a special release sheet is used and is an important feature of the invention. The release sheet to be used is first coated on one side with a pigment, and the pigmented side is placed against the decorative surface prior to the pressure forming of the textured laminate. The color of the pigment is preferably selected to be darker than the color of the decorative sheet or in any event is preferably of a contrasting or highlighting color.

Although any forms of pigment may be employed, the form of pigment used must lend itself to application to the release sheet. For this purpose, therefore, pigments carried in a solvent and binder system capable of being coated onto the release sheet and dried after application are preferred, such as printing inks. It is not necessary to apply the ink to the release sheet in accordance with any pattern, and in fact, a substantially uniform and unpatterned application is preferred to assure complete coverage of the decorative surface. Uniform coating of the ink onto the release sheet by conventional rotogravure methods has been found suitable for this purpose.

The material for the release sheet may be selected from any of the materials in common use and include foil, polymer films and treated paper films. Polypropylene film is especially preferred due to its ability to release the ink when placed under the heat and pressure conditions used in the laminating process.

The components of the decorative laminate, pigmented release sheet and textured caul are then assembled as a sandwich as aforesaid and are compressed in the aforesaid manner at sufficient pressures and temperatures to cause curing and bonding of the resin impregnated sheets. During the laminating process, the textured surface of the caul is imparted to the decorative surface, and at the same time, the release sheet conforms to the irregular surfaces and transfers pigment thereon substantially uniformly onto the decorative surface of the laminate. Upon curing, the release sheet is stripped away from the textured decorative surface, which is now substantially uniformly coated with the pigment.

Under high volume production conditions, it is preferable to use a caul plate having a textured surface on both sides, since an assembly of caul plates and resin impregnated paper assemblies may be compressed and heated simultaneously. For example, five cauls can be used in a single molding operation to produce ten decorative panels.

In the production of a simulated wood panel, wood grain print sheet is utilized, and a wood grain texture is imparted to the laminate. The pattern of the print sheet need not coincide with the texture pattern to produce the desired results, thus eliminating the problem or bringing the patterns into exact register.

The pigmented textured surface of the laminate is now subjected to an operation in which some or all of the pigment remaining on the embossed areas is removed from such areas of the surface while allowing a greater amount of pigment to remain in the debossed areas. This operation may be accomplished by surface rubbing or brushing, exposing the lighter shades of the raised grain or texture and enhancing a three dimensional shadow effect. A suitable procedure is to brush the textured surface with rotary bristle or tampico brushes, preferably in the direction of the grain pattern. Such apparatus is conventionally used in a dull rubbing operation to reduce the gloss of the decorative surface of laminates, and any equivalent procedure for mechanically removing the pigment from the high spots would be effective.

The pigment used preferably will be one having high adherence properties, but in any event it is believed that some of the pigment migrates into the resinous surface, particularly in the debossed areas which are subjected to the greatest molding pressure, and becomes bonded therein as the resin is cured.

The resulting laminate will thus have a textured surface with a greater concentration of pigment in the debossed areas than in the embossed areas. By means of the present invention, therefore, it is possible to create a variety of effects, particularly with the use of contrasting colors in the decorative surface and pigment.

## Claims

1. A method of imparting highlights or shadows to a decorative laminate comprising the steps of preparing a textured decorative laminate by compression molding utilizing a pigmented release sheet to cause transfer of pigment to said laminate, and then rubbing the surface of the pigmented textured laminate to the extent necessary to remove some of the applied pigment, with more pigment being removed from the raised areas of the textured laminate than from the depressed areas thereof.

2. A method of imparting color highlights or shadows to a textured decorative laminate, which comprises the steps of making an assembly of heat curable resin impregnated sheets, placing a release sheet having a pigmented surface against an outer surface of said assembly wherein the pigmented surface is facing said outer surface, compressing and heating said assembly and release sheet under conditions to cure said resin and bond said assembly into a laminate while imparting texture to said outer surface and while causing transfer of pigment from the release sheet to the outer surface, and upon completion of the compression and heating operation, removing said release sheet from the cured laminate to expose the textured, pigmented surface, and then rubbing said surface to the extent necessary to remove more pigment from the raised areas than the depressed areas of said surface.

3. A method as claimed in claim 2, wherein the release sheet is polypropylene film.

4. A method as claimed in claim 2 or claim 3, wherein said pigment is liquid ink applied to said release sheet and dried thereon.

5. A method as claimed in claim 4, wherein said ink is applied substantially uniformly to said release sheet.

6. A method as claimed in any of claims 2 to 5, wherein rubbing the textured, pigmented surface comprises brushing with a rotary brush.

7. A method as claimed in any of claims 2 to 6, wherein said outer surface has a wood grain pattern printed thereon and said pigment is of a shade which contrasts with said outer surface.

8. In conjunction with the production of a decorative laminate having a textured outer surface wherein the laminate is formed by making an assembly comprising resin impregnated sheets, applying a release sheet over an outer surface of said assembly, and forming a laminate by heating and compressing said assembly between a pair of molding cauls, wherein one of said cauls had a textured surface facing said release sheet and serving to impart a textured finish to said outer surface, a method of imparting color highlights or shadows to the outer textured surface of said laminate, said method comprising the steps of providing said release sheet with a pigment coating facing said outer surface such that pigment is transferred from said release sheet to said outer surface during said heating and compressing step and while texture is being imparted to said outer surface, and upon formation of said laminate, removing the release sheet to expose the outer pigmented, textured surface, and rubbing said textured surface such that pigment is removed more from the raised areas than the depressed areas thereof.

## Revendications

1. Méthode pour conférer des effets de lumière ou d'ombre à un stratifié décoratif, méthode caractérisée en ce qu'elle comprend les étapes consistant à préparer un stratifié décoratif texturé par moulage sous pression en utilisant une feuille que l'on peut enlever, pigmentée, pour transférer un pigment sur ce stratifié, et à frotter ensuite la surface du stratifié texturé, pigmenté, dans la mesure nécessaire pour éliminer une certaine proportion du pigment déposée, en retirant plus de pigment des zones en relief des stratifiés texturés que des zones en creux de ces stratifiés.

2. Méthode pour conférer des effets de lumière ou d'ombres à un stratifié décoratif texturé, méthode caractérisée en ce qu'elle comprend les étapes consistant à préparer un assemblage de feuilles imprégnées de résine polymérisable à chaud, à placer une feuille amovible ayant une surface pigmentée sur une surface extérieure de cet assemblage, la surface pigmentée se trouvant face à face avec la surface extérieure, à comprimer et chauffer cet assemblage avec la feuille amovible, dans des conditions où la résine est polymérisée et où l'assemblage est collé pour former un stratifié en provoquant le transfert du pigment de la feuille amovible sur la surface extérieure, à retirer la feuille amovible du stratifié polymérisé, quand les opérations de pression et de chauffage sont terminées, pour mettre à nu la surface texturée, pigmentée, et à frotter ensuite cette surface dans la mesure nécessaire pour éliminer une plus grande quantité de pigment des surfaces en relief que des surfaces en creux de cette surface.

3. Méthode selon la revendication 2, caractérisée en ce que la feuille amovible est une feuille de polypropylène.

4. Méthode selon l'une quelconque des revendications 2 et 3, caractérisée en ce que le pigment est une encre liquide appliquée sur la feuille amovible et séchée sur celle-ci.

5. Méthode selon la revendication 4, caractérisée en ce que l'encre est appliquée sensiblement uniformément sur la feuille amovible.

6. Méthode selon l'une quelconque des revendications 2 à 5, caractérisée en ce que le frottement de la surface texturée, pigmentée comprend un brossage par une brosse rotative.

7. Méthode suivant l'une quelconque des revendications 2 à 6, caractérisée en ce que la surface extérieure porte en impression une apparence de grain de bois, et que le pigment est d'une nuance qui contraste avec celle de la surface extérieure.

8. En relation avec la production d'un stratifié décoratif présentant une surface extérieure texturée, où le stratifié est formé en préparant un assemblage comprenant des feuilles imprégnées de résine, en appliquant une feuille amovible sur une feuille extérieure de cet assemblage, et formant un stratifié en chauffant et comprimant cet assemblage entre deux plaques servant de moules, une de ces plaques ayant une surface texturée venant en face de la feuille amovible et suivant à donner à cette surface extérieure un fini texturé, méthode pour conférer des effets colorés de lumière ou d'ombres à la surface extérieure texturée du stratifié, cette méthode comprenant les étapes consistant à garnir la feuille amovible d'un revêtement de pîgment faisant face à cette surface extérieure de telle façon que le pigment soit transféré de la feuille amovible sur cette surface extérieure au cours de l'étape de chauffage et de compression et pendant qu'une texture est donnée à la surface extérieure, à retirer la feuille amovible après formation du stratifié, pour mettre à nu la surface extérieure pigmentée, pour mettre à nu la surface extérieure pigmentée, texturée, et à frotter la surface texturée de manière à enlever plus de pigment des zones en relief que des zones en creux de cette surface.

## Patentansprüche

1. Verfahren zum Verleihen von Glanz oder Schatten an einen dekorativen Schichtstoff, welches die Schritte umfaßt, daß ein texturierter dekorativer Schichtstoff durch Preßformen vorbereitet wird, daß eine pigmentierte Freigabebahn verwendet wird, um die Übertragung von Pigment auf den Schichtstoff herbeizuführen, und daß die Oberfläche des pigmentierten texturierten Schichtstoffs in dem Ausmaß gerieben wird, das erforderlich ist, um etwas von dem aufgebrachten Pigment zu entfernen, wobei mehr Pigment von den erhabenen Bereichen des textureierten Schichtstoffs als von seinen vertieften Bereichen entfernt wird.

2. Verfahren zum Verliehen von Farbglanz oder Schatten an einen texturierten dekorativen Schichtstoff, welches die Schritte aufweist, daß eine Anordnung aus mit Wärme härtbaren harzìmprägnierten _{`} Bahnen angefertigt wird, daß eine Freigabebahn, die eine pigmentierte Oberfläche hat, an einer äußeren Oberfläche der Anordnung plaziert wird, wobei die pigmentierte Oberfläche der äußeren Oberfläche zugewandt ist, daß die Anordnung und die Freigabebahn unter Bedingungen komprimiert und erhitzt werden, bei denen das Harz härtet und die Anordnung zu einem Schichtstoff gebunden wird, während der äußeren Oberfläche eine Textur verliehen wird und während die Pigmentübertragung von der Freigabebahn zu der äußeren Oberfläche veranlaßt wird, und daß nach Vervollständigung des Komprimier- und Erhitzungsvorgangs die Freigabebahn von dem gehärteten Schichtstoff entfernt wird, um die texturierte pigmentierte Oberfläche freizulegen, und daß dann die Oberfläche in einem Ausmaß gerieben wird, das erforderlich ist, um mehr Pigment von den erhabenen Bereichen als von den vertieften Bereichen dieser Oberfläche zu entfernen.

3. Verfahren nach Anspruch 2, bei welchem die Freigabeschicht eine Polypropylen-Folie ist.

4. Verfahren nach Anspruch 2 oder 3, bei welchem das Pigment flüssige Farbe ist, due auf die Freigabebahn aufgebracht und darauf getrocknet ist.

5. Verfahren nach Anspruch 4, bei welchem die Farbe im wesentlichen gleichförmig auf die Freigabebahn aufgebracht wird.

6. Verfahren nach einem der Ansprüche 2 bis 5, bei welchem das Reiben der texturierten, pigmentierten Oberfläche aus einem Bürsten mit einer Drehbürste besteht.

7. Verfahren nach einem der Ansprüche 2 bis 6, bei welchem die äußere Oberfläche ein aufgedrucktes Holzmaserungsmuster aufweist, und das Pigment eine Schattierung hat, die mit der äußeren Oberfläche in Kontrast steht.

8. Mit der Herstellung eines dekorativen Schichtstoffs mit einer texturierten äußeren Oberfläche, wobei der Schichtstoff dadurch gebildet wird, daß eine Anordnung erzeugt wird, welche harzimprägnierte Bahnen aufweist, eine Freigabebahn über eine äußere Oberfläche der Anordnung gelegt wird und ein Schichtstoff durch Erhitzen und Komprimieren der Anordnung zwischen einem Paar von Formplatten gebildet wird, von denen eine eine texturierte Fläche hat, der Freigabebahn zugewandt ist und dazu dient, der äußeren Oberfläche ein texturiertes Finish zu verleihen, in Verbindung stehendes Verfahren zum Verleihen von Farbglanz oder Schatten an die äußere texturierte Oberfläche dieses Schichtstoffs, wobei dieses Verfahren die Schritte aufweist, daß die Freigabebahn mit einem Pigmentüberzug versehen wird, welcher der äußeren Oberfläche zugewandt ist, so daß Pigment von der Freigabebahn auf die äußere Oberfläche während des Erhitzens und Komprimierens und während der äußeren Oberfläche die Textur aufgeprägt wird, übertragen wird, und daß nach der Bildung dieses Schichtstoffs die Freigabebahn entfernt wird, um die äußere pigmentierte texturierte Oberfläche freizulegen, und daß die texturierte Oberfläche derart gerieben wird, daß mehr Pigment von den erhabenen Bereichen als von den vertieften Bereichen entfernt wird.
